

Patented July 28, 1925.

1,547,453

# UNITED STATES PATENT OFFICE.

LEO L. SIMON, OF NEW YORK, N. Y.

## ORNAMENTAL FEATHER.

No Drawing.

Application filed July 5, 1924. Serial No. 724,519.

To all whom it may concern:

Be it known that I, LEO L. SIMON, a citizen of the United States, residing at New York, in the county of New York and State of New York, have invented certain new and useful Improvements in Ornamental Feathers, of which the following is a specification.

This invention relates to the treatment of feathers and to the articles that results from such treatment.

One of the objects of this invention is to prepare feathers such as are used for ornamental purposes on women's hats and the like in such a manner as to increase their wearing qualities or their durability.

Another object of this invention is to treat such feathers in such a manner as to increase their ornamental value and quality.

It is also an object of my invention to provide a process which will make it possible to vary the ornamental quality of feathers.

These objects are accomplished by the steps described hereinafter severally or jointly. Some of the steps have for their object the stiffening of the feathers to the result that the durability and wearing quality of the feathers are increased. Other steps described hereinafter have for their object the application of a variegated colored surface to the feather with the result that its ornamental quality is increased. Moreover with the process described herein-after the same type of feather may be treated in different manner so as to give it entirely different appearances with the result that the same type of feather may be used with different types of millinery or other garments. In my process the feather is first coated with varnish and allowed to dry. This stiffens the feather and increases its wearing qualities and its durability. If desired, the feather may be sold and used in this form.

For the purpose of applying a variegated colored coating to the feather the next step is to apply one or more coats of paint or enamel to the feather. This coating of paint or enamel may be of any desired color and constitutes the base or basic color of the variegated color combination aimed at. The number of coats of paint or enamel to be applied during this step vary with the

effects desired and vary with the degree of stiffening desired and the quality of the feather. After the last coat of paint or enamel has been thoroughly dried a crackling enamel is applied. The crackling enamel is of such a nature that when it dries it cracks, with the result that it represents a number of spots of one color applied to a ground of a different color. The crackling enamel obviously must be of a color different from the color of the previous coat. The result is a variegated colored surface on the feather. These surfaces and color combinations obviously may be varied in any manner desired and may be made in such form as to imitate various artificial or natural objects such as various leather or animal skins or the like.

The result is an article in the shape of a feather, sometimes obviously a feather which may look like an alligator skin for example, or anything else desired.

Instead of using crackling enamel any ordinary enamel may be used, but it must be applied with a stippling brush or be applied in such a manner as to give a stippled effect. In other words, the last coat of enamel must be applied in such a manner as to give the resultant effect of spots of enamel or paint of one color superposed upon a groundwork of enamel or paint of a different color.

Another method of obtaining the variegated color effect which may be used is to apply the last coat of enamel of a color different from the preceding coat of enamel while the preceding coat is still wet and to cause the two coats of enamel to flow and intermix in such a manner as to bring about the desired variegated effect.

Applicant does not wish to limit himself to any specific method of obtaining the variegated color effect on the surface of a feather.

After the crackling enamel has been dried or after the variegated effect has been completed and dried, one or more coats of a plain color varnish or enamel are applied to the surface so as to give the article a bright finish and also to protect the crackling finish from direct exposure to weather and from wear.

The product obtained as a result of this process is a feather which may be used for

ornamentation on women's hats or the like which is stiff and will not bend or break on exposure to the winds as readily as feathers used hitherto for such purposes and will 5 wear better than other feathers.

The process disclosed herein may be applied to other materials.

What is claimed is:

1. An article of manufacture comprising 10 a stiffened feather having a layer of paint thereon and a protective coating to protect the paint.

2. An article of manufacture comprising 15 a stiffened feather having a layer of variegated colors thereon and a coating for protecting said layer.

3. An ornamental article for wearing apparel comprising a body of soft fluffy material having an initial stiffening layer 20 thereon, an ornamental layer of paint or enamel and a protective layer.

4. The process of treating feathers com-

prising the step of applying a coating of a stiffening agent thereto.

5. The process of treating feathers comprising the steps of applying a stiffening coating to the feather and applying a variegated colored coating to the feather.

6. The process of treating feathers comprising the steps of applying a variegated 30 colored coating thereto and of applying a protective coating thereto.

7. The process of manufacturing an ornamental article out of soft fluffy material comprising the steps of applying a layer 35 of varnish thereto, a layer of enamel and a layer of crackling enamel.

8. The process described in claim 7 in which a protective coating of enamel is applied over the crackling enamel.

In testimony whereof I hereunto affix my signature.

LEO L. SIMON.